

June 24, 1930.

L. KIRSCHBRAUN

1,767,374

METHOD OF MAKING ROOFING ELEMENTS

Original Filed Aug. 24, 1925 2 Sheets-Sheet 1

Fig. 1.



Fig. 2.



Fig. 3.



Fig. 5.



Fig. 6.



Fig. 4.

By Wright, Brown, Quincy & May

Attorneys

Inventor

Lester Kirschbraun

June 24, 1930.

L. KIRSCHBRAUN

1,767,374

METHOD OF MAKING ROOFING ELEMENTS

Original Filed Aug. 24, 1925 2 Sheets-Sheet 2



Fig. 7.



Fig. 8.

Inventor  
Lester Kirschbraun

By Wright, Brown, Quincy & May

Attorneys

## UNITED STATES PATENT OFFICE

LESTER KIRSCHBRAUN, OF LEONIA, NEW JERSEY, ASSIGNOR, BY MESNE ASSIGNMENTS,  
 . TO THE PATENT AND LICENSING CORPORATION, OF BOSTON, MASSACHUSETTS, A  
 CORPORATION OF MASSACHUSETTS

## METHOD OF MAKING ROOFING ELEMENTS

Continuation of application Serial No. 134,412, filed September 9, 1926, which is a division of application Serial No. 51,949, filed August 24, 1925. Patent No. 1,612,776, dated December 28, 1926. This application filed October 8, 1929. Serial No. 398,232.

This invention relates to the production of roofing elements generally of the character of shingles, slabs, shingle strips, clapboard or the like, in which, when the material is laid upon the roof in overlapping courses, there are exposed marginal portions with edges that are subject to deterioration caused by the sunlight and the elements, the subject matter of this application being a continuation of my copending application Serial No. 134,412, filed September 9, 1926, which in turn is a division of my copending application Serial No. 51,949, filed August 24, 1925, upon which Letters Patent No. 1,612,776 were granted to me Dec. 28, 1926.

Ordinarily, in the manufacture of modern roofing such as employed for these purposes, it is the custom first to form a sheet of felt which is made ordinarily of rag fibers or 20 rag and asbestos fibers or the like, of the desired caliper and of sufficient porosity to permit it to absorb a molten waterproofing composition such as pitch, asphalt or the like, and of sufficient strength to enable it 25 to be manipulated during the operations of forming the ultimate roofing product. This is a common article of commerce which is ordinarily known as roofing felt and is produced on the usual paper-making machines. 30 After the sheet has been properly saturated with the bituminous saturating compound, either by immersion in a bath of a molten bitumen or pitch, or by subjection to "pressure saturation", the sheet is coated on one 35 face with a fairly thin layer of high melting-point asphalt. For this purpose, oxidized or blown asphalt so-called is preferably employed because of its tough and rubbery nature. While the asphaltic coating is 40 still soft and plastic and before it has set, it is surfaced with any suitable form of crushed mineral such as crushed slate, tile or any other mineral grit which will impart the desired color and texture to the final 45 product. The grit is preferably formed in relatively large particles or granules which vary in form according to the material from which they are produced. The surface mineral coating is partially embedded in the 50 plastic asphaltic coating sufficiently to in-

sure a firm interlocking of the granules with the asphaltic coating, but leaving the granules so exposed that the asphaltic layer is completely covered and masked by the particles or grains of grit. In ordinary practice 55 the sheet thus formed is now cut into roofing elements, which take the form of individual shingles or strip shingles or slabs of various designs or in long narrow strips which may be employed for the sides of buildings in the 60 same manner as wooden clapboards.

The operation of the cutting machinery is such that, when these roofing elements are produced, at all of the edges of the element there are exposed first the saturated felt, 65 next a thin stratum of asphalt, and finally the layer of grit the grains of which are partially embedded in the asphalt.

It has been discovered that asphalt exposed to the elements and to the sunlight is 70 susceptible to rapid deterioration. It is known, for example, that the action of sunlight or of the ultra violet rays is such as to cause a condensation of polymerization of the asphalt, resulting in the hardening of 75 the asphalt with a consequent checking or breaking down of the asphalt particularly when it is exposed in relatively thin films or layers. This is especially true of the asphalt or other bitumen which is utilized as the 80 saturating compound for the foundation felt, inasmuch as the films of asphalt about the fibers of the felt are relatively thin. Due to the action of the light and of moisture, these films crumble; and this, together with 85 the absorption of moisture by the exposed fibers, causes the breaking down of the exposed edges and produces a tendency on the part of the exposed margin of the roofing element to curl. The curling is doubtless 90 also accelerated by the fact that the layer of coating asphalt contracts under the influence of the elements and the rays of the sun and because of oxidation to a greater extent than the saturated felt itself.

On the other hand, a single layer of asphalt which is too thick is liable to crack through from internal stresses set up by unequal heating and cooling, especially in 100 winter weather when the asphalt is com-

paratively hard and brittle. Cracks thus formed in a coating of asphalt admit moisture to the fibrous foundation of the element which is absorbed and tends to bulk or swell the felt. This, especially in conjunction with frost, tends to disintegrate the element by warping it, loosening the asphalt coating and extending the original crack or fissure. To secure best results in 10 weatherproofing with a single coating of "blown" asphalt, such coating should be from .040 to .070 of an inch thick. The grit surfacing material usually applied to such a coating often comprises particles large enough to extend all the way through the 15 coating and puncture it. If these particles are dislodged in the subsequent treatment and handling of the roofing, they leave small pin-holes in the coating, through which moisture can enter. While these breaks in 20 the continuity of the surface coat are not as serious a cause of deterioration of the element as are the cut exposed edges, yet their tendency is in the same direction, 25 namely, to shorten the life of the element. An extra coating of asphalt over the surface of the element which is exposed when laid closes all such pin-holes and other possible breaks in the first coating. Although the 30 second coating infiltrates between the particles of grit and bonds with the first coating, the grit layer maintains the separate identity of the two coatings and prevents the cracking stresses which would ordinarily be set up by thermal changes in a single 35 layer of coating material of a thickness equal to the sum of the two coatings.

In the practical production of the roofing elements herein referred to, it is customary 40 to apply the grit surface layer to only one face of the product, a portion of which is to be exposed to the weather, and in most cases the under face of the roofing elements consists of merely the saturated felt. In some 45 instances it is true that a thin layer of the asphaltic coating is applied to the under face of the roofing element when the sheet is being saturated and coated. When the elements are laid in overlapping courses, 50 however, water finds its way under the exposed edges and margins of the elements, either by capillary action or by the beating rain with the assistance of the wind, and in winter weather this moisture freezes and 55 thaws and has the effect of lifting the exposed edges of the roofing elements from contact with the elements overlapped thereby, so that the deterioration of the asphalt hereinbefore referred to is localized 60 not only at the edges of the roofing element but also extends through the under face thereof with the consequent tendency to disintegration and destruction of the foundation sheet. This is true even in cases 65 where the under face of the product is

coated, for the reason that ordinarily such coatings are so thin that they are rapidly attacked and their efficiency destroyed.

The problem which thus presents itself is to find some way of preventing or overcoming the deterioration at the cut edges 70 of the roofing material and of prolonging the effective life of such roofing elements. In attacking this problem, one is confronted with the fact that the saturated felt is the weakest component of the roofing product so 75 far as its liability to deterioration is concerned. The cellulosic fibers of which it is formed have an affinity for moisture, and the saturated felt itself ordinarily will absorb moisture up to 20% of its weight. Yet the integrity and the strength of the roofing product are directly dependent upon the integrity and strength of the saturated felt, for if this be destroyed the product as 80 a whole loses its waterproofing and durable characteristics. The deterioration of the saturated felt is evidenced by progressive loss of cohesiveness and structural strength, so that the resistance of the final product to 85 the weaving of the roof structure and its flexing through the action of the winds and the elements becomes insufficient to maintain it in place.

In seeking an answer to the problem, 90 therefore, means must be provided for the maximum protection of the saturated felt to prevent access of moisture, oxygen and light thereto. This is accomplished by providing what may be termed a supplemental 95 coating of high melting-point asphalt, preferably blown asphalt, in a layer of sufficient thickness so as completely to seal the fibers of the felt with an impermeable envelope so as to prevent the access of air or moisture; 100 but, inasmuch as asphalt itself is subject to deterioration through the action of light as hereinbefore stated, the impermeable asphaltic envelope itself is liable to deterioration and destruction. Consequently to overcome 105 this defect, means must be afforded for preventing the access of light to the asphaltic layer. This is accomplished by enclosing the asphaltic layer within an opaque 110 layer. Any suitable opaque material may 115 be utilized for this purpose, but as a practical matter one may employ crushed slate, crushed tile, or any other opaque granular material which may be partially embedded in the asphaltic layer in such manner as completely to cover it and to prevent the access 120 of the rays of the sun directly thereto to any substantial extent.

The present invention comprises an individual roofing element in the nature of a shingle, shingle slab or strip, having the exposed edges sealed by an enclosing envelope of asphalt or bitumen and the envelope itself is protected against light by a surface 125 130

layer of an opaque material preferably applied in granular form.

Incidentally, however, I have found that it is possible to produce a roofing material which is superior to those heretofore made of flat sheets, in that the element may be so formed that it is gradually thickened towards what may be called the butt or exposed end thereof. Thus, when the roofing elements are laid in overlapping courses, the roof thus formed has the appearance of and has an actual degree of thickness which imparts a pleasing effect and which relieves such roofs from the monotony and flatness that have characterized roofs formed of flat elements.

A roofing element thus formed possesses certain other highly desirable characteristics which are lacking in the ordinary flat element as heretofore produced. First, by reason of the fact that the element is thickest at the butt or exposed edge thereof, its weight is greatest at the edge and consequently the exposed edge offers greater resistance to the lifting force of the wind and will remain flat when the flat elements of unvarying thickness would be lifted or raised by the wind's pressure. This also permits of greater area of exposure. Again, inasmuch as both faces (that is, the upper and the lower faces) of the element are coated to substantially the same extent by the asphaltic envelope, there is no tendency for the exposed portion of the element to curl away from the element overlapped thereby. Asphalt, when exposed to light and the elements, tends to contract; and, where the roofing element has no or only a thin layer of asphalt on its under side and a relatively thick layer on its exposed side, the contraction of the exposed layer causes the curling of the entire element. This is observable on many roofs which have been covered with flat individual slate-surfaced shingles.

In the production of such elements as herein described, one may start with the ordinary roofing elements of commerce, namely, individual shingles, strip shingles or slabs, or clapboard slabs, all of which are designed to be laid in overlapping courses with what may be termed for convenience exposed butt portions. These butt portions are dipped into a bath of molten asphalt for a sufficient time to cause them to be covered on both faces and on their exposed edges with a fairly thick layer of asphalt. On removing the elements from the asphaltic bath, they are permitted to hang vertically and drain sufficiently to permit the excess asphalt to drop therefrom and to permit a flow of the attached coating so that it is thickest at the pendent edge of the element. While the coating is still soft and plastic, it is coated on both faces and on its edges with a layer of opaque granular material,

the grains of which are partially embedded in the asphaltic coating but protrude therefrom so as to completely cover and mask the asphaltic envelope.

On the accompanying drawing I have illustrated a strip shingle embodying the invention, but it will be understood that the invention may equally well be incorporated or embodied in an individual shingle, or a clapboard strip.

Figure 1 represents a shingle strip as ordinarily formed, and which in the present instance serves as the starting material of my product.

Figure 2 represents the completed product.

Figure 3 represents a section on the line 3—3 of Figure 2.

Figure 4 represents an enlarged section on the line 4—4 of a part of the strip shingle.

Figures 5 and 6 illustrate the formation of a double-dipped shingle.

Figure 7 represents in perspective a tank in which shingles may be dipped.

Figure 8 represents a receptacle for grit or other comminuted material by which the dipped shingle is surfaced.

Referring to the drawing, I have shown in Figure 1, at *a* what is commercially known as a slate surfaced square butt strip shingle, which is provided at *b*, *b* with tabs or projections and intervening notches *c*, *c*. Such a shingle is usually laid with others in overlapping courses, so that the butts of the tabs register with the upper ends of the notches of the strips overlaid thereby. The tabs may, for example, be four inches in length, where the entire strip is ten inches between its upper and lower edges. Of course it will be understood that the design of the strip shingle may be varied, so that the tabs may be semi-hexagonal, or semi-octagonal, or of any other desired shape.

The shingle strip, as shown, has a base of rag or asbestos felt 10, which is impregnated with asphalt or other commonly used waterproofing compound, a layer 11 of higher melting-point asphalt, and a surface layer 12 of granular material.

The strip is held by its straight upper edge, and is dipped into a bath of molten asphalt, which is preferably oxidized or blown asphalt having a melting point of 220°-240° F. The dipping operation must be carried on while the molten asphalt is at an elevated temperature, and is so timed that the strip will pick up the proper amount of asphalt and also readily free itself of the excess. If a heavy coating is desired, the temperature of the bath is lower than when a thinner coating is to be applied. I have found that the desirable temperature to produce the optimum viscosity of the asphalt is in the range of 425°-450° F. when using oxidized asphalt from Mexican stock. It

will be appreciated that the viscosity of an oxidized asphalt at a given temperature, will vary with the nature of the stock from which it is prepared, as well as its melting point, and the temperature to which it is heated. Therefore the temperature range which I have given is only indicative of the viscosity of the particular stock there referred to. The period in which a part of the shingle strip is dipped in the asphalt must be very short in order not to melt or unduly heat or soften the underlying bituminous material unnecessarily. One or two seconds is usually sufficient.

The shingle strip is dipped in the bath far enough to cause the molten asphalt to cover all of that portion of the strip which will be exposed when it is laid, usually to a longitudinal line parallel to the upper edge of the strip about half an inch to an inch above the ends of the notches. The strip is removed from the bath and while hanging is permitted to drain momentarily to permit the coating on both faces to flow toward the lower edge, and thus form tapered layers which are thickest at the edge, the excess drops being "flipped" or else wiped off. The process thus far described may be carried out manually by the use of a suitable pool of molten asphalt contained in a tank which is of sufficient length to receive the strip shingle. The asphalt may be maintained at the desired temperature by any suitable heating means, such as steam coils disposed near the bottom thereof. In order to wipe the dripping asphalt from the butt edge of the dipped shingle, wiping elements such as steam pipes, may be provided at convenient locations as shown in Figure 7. The strip is now surfaced with an opaque grit which is caused to become partially embedded in the still plastic asphaltic coating or envelope, not only on the faces of the strip but on all the edges thereof which are asphalt-coated, and as a consequence there is a continuous layer of exposed grit which extends over both faces and across all of the lower edges of the strip, including the edges of the tabs and the edges at the upper ends of the cutouts or notches. This may be done by first pressing the strip flatwise against a thick layer of loose grit, which may be conveniently located in a suitable box or container, then rocking the strip through an arc of  $180^{\circ}$  about its asphalt-coated lower edge as the center as indicated in Figure 8, and pressing the other face against the layer of loose grit, and forcing or piling grit into the cutouts or recesses and against the end edges of the strip. This molds the asphalt and grit at the lower edge of the strip and furnishes a straight rounded edge which is pleasing in appearance. The strips are piled one on the other, as produced, and the weight of the pile forms flat

surfaces on the faces of the strips. The operations may, however, be performed by suitable automatic machinery.

In Figure 2 of the drawing, I have shown the slate-surfaced strip shingle of Figure 1, as it appears when it has been subjected to the operations herein described. It will be noted from the sectional view illustrated by Figure 3, that the shingle strip is thickest at its butt or lower edge, and tapers upwardly to a line just about the cut-outs or recesses.

In some cases for the opaque granular material, which is employed to cover, protect and mask the asphaltic envelope, I prefer to employ grit or granules of a different color and/or size from those which originally formed the outer layer of the original strip, especially in the case of strip shingles or individual shingles, so that a contrast will be afforded between the exposed portions thereof and the upper portions of the overlapped strips, which are visible through the notches, or through the spaces between the individual shingles. Again, instead of starting with a grit-coated roofing element, as hereinbefore described, one may start with a roofing element cut from "rubber roofing", so-called, which is an asphalt-impregnated sheet, having layers of high melting-point asphalt on one or both faces thereof. Usually, but not necessarily, such "rubber roofing" has a surface layer of talc or mica.

I should not regard it as a departure from my invention if the protecting asphaltic envelope of the roofing elements were surfaced with pulverized material, or with talc or mica, or if the envelope itself were formed of a colorable pitch such as stearin pitch, or mixtures of resins and tempering fluxes, with a suitable pigment incorporated therein to impart the desired color thereto.

In instances where it is desired to keep down the weight of the roofing element, the front face and the edges of the strip may be surfaced with crushed slate partially embedded in the asphaltic envelope, and the rear face surfaced with a fine powder such as talc or mica.

In certain cases where an extra thick butt is desired on the roofing element, I may subject the element to a series of dipping and grit-surfacing operations. In such case, in the first dipping the element may be immersed, say, one and one half to two inches, and after the grit-surfacing operation has been carried out, and the asphaltic coating has set, the element is in the second dipping immersed to an extent of five inches, after which it is surfaced, covered and protected with a layer of granules of opaque material.

In Figures 4, 5 and 6, I have shown a strip which has been subjected to the series of operations last described.

5 In order to secure certain results, one may surface the edges of the cut-outs or recesses of a shingle strip with "fines" of the same color as the granules which coat the faces of the strip. Such "fines" are the powders or dusts which separate from the larger granules of slate or other mineral grit.

10 In each of the roofing elements herein described, the continuous asphaltic coating which covers the upper and under faces and the bottom and side edges of the exposed or butt portion thereof, is securely interlocked with the usual granular facing, if there be one, on the upper face of the element, and 15 more or less coalesces with the asphaltic impregnating compound at the edges and on the under faces of said butt portion. While the period of immersion or dipping is very short so as not to melt such impregnating compound and the initial asphaltic coating, yet there is sufficient heat in the second or continuous coating to cause a sufficient softening thereof and to cause the necessary coalescence and interlocking of the two.

20 I claim:

25 1. A method of making roofing elements, which comprises dipping the butt portion of a previously formed element, having an asphaltic coating and a layer of partially embedded granular material on one face thereof, into a bath of molten asphalt, withdrawing the element and suspending it in an upright position for a brief period with its butt edge down, and applying a granular material to the coating thus formed while it is soft and plastic.

30 2. A method of making roofing elements, which comprises applying a coating of molten asphalt to the butt edge of a pre-formed element, placing said butt edge in contact with grit while the asphalt is still hot and sticky, and rocking the element on the butt edge as an axis while said edge is in contact with said grit.

35 3. A method of making roofing elements, which comprises applying a coating of molten asphalt to the faces and edges of the butt portion of a pre-formed element, bringing one face of said element in contact with grit while the asphalt is still hot and sticky, and rocking said element on the butt edge as an axis, said butt edge being in contact with grit during said rocking.

40 4. A method of making roofing elements, which comprises dipping the butt portion of a pre-formed element into a bath of molten asphalt, withdrawing the element and permitting the asphalt to flow toward the butt edge, applying a face of the ele-

45 ment to a body of loose grit, and rocking said element on said butt edge while the latter remains in contact with said body of grit.

50 5. A method of making roofing elements, which comprises enveloping the butt portion of a pre-formed element completely

55 with a coating of molten asphalt, applying one face of said element to a body of grit, and rocking said element on the butt edge as an axis until the opposite face comes in contact with the grit, the butt edge being in contact with the grit during the rocking of the element.

60 6. A process for making prepared roofing which resides in notching the edge of a base of roofing material, in depositing a waterproofing composition on the surface of said base to coat the butt edge thereof, in suspending the base to position its upper edge above the plane of the butt edge thereof to cause the waterproofing composition to flow over the surface of the shingle and gradually increase in thickness towards its notched edge and in applying granular material to said waterproofing coating.

65 7. A method of manufacturing prepared roofing, comprising notching one edge of a roofing base to form a series of shingle simulating tabs on said base, coating a face of the base and the butt and side edges of the tabs while maintaining the butt edge of the base at a lower plane than the opposite edge thereof, to cause the coating to drain downwardly to increase the thickness of the coating retained on the base towards the notched edge thereof and applying to the coated portion of the base granular matter to be retained thereon.

70 8. A method of manufacturing prepared roofing comprising notching one edge of the roofing base to form a series of shingle simulating tabs on said base, coating a face of the base and the butt and side edges of the tabs while maintaining the butt edge of the base at a lower plane than the opposite edge thereof, increasing the thickness of the coating retained on the base toward the notched edge thereof by suspending the base in a position wherein the coating flows by gravity toward the notched edge and applying to the coated portion of the base granular matter to be retained thereon.

75 9. A process for manufacturing roofing strips having a notched edge to provide shingle simulating tabs, comprising retaining one edge of the strip at a plane beyond the notched edge thereof while coating a portion of a face of the strip and the butt and side edges thereof, suspending the strip to cause the waterproofing coating applied thereto to gradually increase in thickness by gravity flow thereof toward the notched edge of the strip and applying granular material to the coated portion of the shingle strip.

80 10. A process for manufacturing roofing strips having a notched edge to provide shingle simulating tabs comprising the steps of retaining one edge of the strip at a plane beyond the notched edge thereof while coating a portion of a face of the strip, suspend-

70

75

80

85

90

95

100

105

110

115

120

125

130

ing the strip to cause the waterproofing coating applied thereto to gradually increase in thickness by gravity flow toward the notched edge of the strip and shaping the coating accumulating on the lower edge of the strip to present a predetermined contour.

11. A process for making shingle strips having tab portions simulating individual shingles, consisting in coating the butt portions of said strips with a waterproofing composition to cover portions of the faces and the edges thereof to be exposed, in thereafter causing said strips to hang in a position to permit the asphalt to flow by gravity and to accumulate in a layer increasing in thickness toward the butt edge of the strip, in smoothing the butt edge of the strip, and in thereafter applying granular material to the coated portion of the strip.

12. A method of making roofing which consists in applying a waterproofing coating to an exposed surface of the base and in suspending said base in a position whereby the coating will flow toward the lower edge thereof and gradually increase in the thickness toward said lower edge and in applying comminuted material to the coated portion of the base.

13. A method of making roofing which consists in applying a waterproofing coating to the exposed surfaces of a base, in suspending said base in a position whereby the coating will flow toward the lower edge thereof and gradually increase in thickness toward said lower edge and in applying comminuted material to the coated portion of the base.

14. In a method of manufacturing roofing wherein a base is notched to form shingle simulating tabs and is thereafter coated with waterproofing material over its exposed faces and edges, the improvement consisting in suspending the notched edge in a lower plane than the opposite free edge thereof to cause the coating to gradually increase in thickness toward the notched edge and in thereafter applying granular material to the coated surface.

15. A process for making roofing strips comprising the steps of notching one edge of the base of material of uniform thickness to form a strip having shingle simulating tabs, coating a surface of the tabs and the butt and side edges thereof with waterproofing bitumen to seal the exposed edges and face of the shingle against weather deterioration, varying the thickness of the coating toward the butt edge thereof to thereby form a thickened and tapered butt edge and thereafter applying comminuted material to the thus coated and tapered exposed surface and the sealed butt and side edges thereof.

16. The process of making thick butt shingles which comprises the steps of suc-

cessively subjecting said shingle to the application of waterproofing bitumen with each successive application extending to a greater distance from the butt edge thereof than the preceding application, and maintaining one edge of said shingle at a plane lower than the other edge whereby the waterproofing bitumen gravitates downwardly to form a tapered butt shingle.

17. A method of making roofing which consists in applying a waterproofing coating to an exposed surface of a base, suspending said base in a position whereby the coating will flow toward the lower edge thereof and increase in thickness toward the lower edge, and in subsequently applying another waterproofing coating to the exposed surface of said base.

18. A method of making roofing which consists in successively applying a waterproofing coating to an exposed surface of a base, with each application of bitumen extending a different distance from the lower edge of the base than the preceding applications whereby the butt edge may be built up to a predetermined thickness, suspending said base following one of said applications of bitumen in a position whereby the coating will flow toward the lower edge thereof and gradually increase in thickness toward said lower edge, and in finally applying comminuted material to the coated portion of the base.

19. A process for making roofing strips from base material of uniform thickness comprising the steps of coating a surface of the base including butt and side edges thereof with waterproofing bitumen to seal the exposed edges and the face of the shingle against weather deterioration, varying the thickness of the coating toward the butt edge thereof to thereby form a thickened and tapered butt edge and in thereafter applying comminuted material to the thus coated and tapered exposed surface and the sealed butt and side edges thereof.

Signed at East Rutherford in the county of Bergen and state of New Jersey, this twenty-third day of September, A. D. 1929.

LESTER KIRSCHBRAUN. 115

70

75

80

85

90

95

100

105

110

115

120

125

130